

Feb. 21, 1956

J. D' A. CLARK

2,735,762

WOOD PULPING PROCESS

Filed Sept. 24, 1953

2 Sheets-Sheet 1



INVENTOR:  
*James D'A. Clark.*  
BY  
*James M. Dougall, William H. Herk,*  
ATTORNEYS.

Feb. 21, 1956

J. D' A. CLARK  
WOOD PULPING PROCESS

2,735,762

2 Sheets-Sheet 2

Filed Sept. 24, 1953

*Fig. 2*



INVENTOR:  
*James d'A. Clark*  
BY  
C. M. McDougal, Williams & French,  
ATTORNEYS.

# United States Patent Office

2,735,762

Patented Feb. 21, 1956

1

2,735,762

## WOOD PULPING PROCESS

James d'A. Clark, Longview, Wash.

Application September 24, 1953, Serial No. 382,065

10 Claims. (Cl. 92—6)

This invention relates to the conversion of woody material to release pulp fibers for use in the manufacture of papers, boards and other felted fibrous structures, and it relates more particularly to a pulping process which releases fibers from woody material in a more efficient and economical manner without deterioration of the fibers or loss in the strength properties thereof to enable use in the manufacture of lower cost and higher strength fibrous structures.

To the present, various means have been used to reduce woody material to particle sizes suitable for digestion by chemical reactions for the elimination of ligneous binders and release of the fibers as pulp for the preparation of fibrous structures. Little attention has been given to the manner in which the woody material has been disintegrated for reduction to particle sizes suitable for digestion with cooking liquors.

It has been found in recent investigations that in the use of conventional devices for disintegration, the wood is crushed or bruised particularly in zones beneath the new surfaces formed upon division and that the degree of crushing is out of proportion with the extent of reduction in particle size.

Recent investigations have also established quite conclusively that the cooking liquors used in the digestion processes tend to attack the cellulosic materials in the bruised areas more violently than the remainder with the result that wooden elements containing bruised portions have been found to produce inferior pulp and the fibrous structures fabricated therefrom have been found to embody less strength as compared to the use of particles containing lesser proportions of bruises. Green and Yorston (Pulp and Paper Magazine of Canada, 41, No. 2: 123-126 February 1940) have found that fibrous chips which have been partially crushed in the manner described during preparation and prior to cooking produce pulp having about one-half the tensile or burst strength, about one-third the tearing strength and about one-twentieth the folding endurance as compared to pulp formed of wooden chips which have been prepared without crushing. Crushing which causes degradation of the type described in wood fibers has been found to result also if thin slices of wood for digestion are planed or sliced from a block of wood with the cutting edge placed at right angles to the grain and moved along the grain. Degradation in such fibrous elements occurs mostly adjacent the side of the slice away from the block and is believed to result from the crushing of the slice by compression of the woody material on the side toward which the slice curls. Although the compression is gentle, such unbelievable losses in strength result that little doubt remains as to the degradation of the fibers which takes place in this form of planing process.

These results have been confirmed in actual practice but the reason for the deterioration of pulp from such material has been attributed to other factors. When the size of the chips is reduced, such as to below  $\frac{3}{8}$  inch, the quality of the resulting pulp has been found to commence to deteriorate substantially. The inclusion of fines, such as sawdust, has been found to reduce the quality of the pulp very severely. The industry has advanced various theories for the deterioration in the characteristics of pulp made from fine wood particles; most of the theories have centered upon the concept that harmful results are se-

2

cured because of excessive cutting of the fibers in the wood and the adverse effect of the fine material upon liquor circulation. Now it appears that the principal factor resides in the discovery of the adverse effect of bruising and crushing which increases in proportion inversely with the size of the wooden particle.

Because of the misleading hypotheses with respect to chipping which have in the past been accepted by those skilled in the art, there has been no incentive to search for means for greater size reduction notwithstanding the apparent economies and efficiencies in operation based upon the more rapid penetration of the cooking liquor into the smaller particles with a yield of a more uniform pulp.

Another reason for the persistent adherence to present practice in chipping and cooking woody materials in the manufacture of pulp has been the unavailability of devices of sufficient capacity for effecting size reduction without excessive damage to the fibers in a practical and yet economical manner.

It is an object of this invention to provide a new and improved method for reducing woody material in the manufacture of pulp and it is a related object to provide a continuous process for achieving same while preserving the inherent strengths of the pulp fibers.

Another object is to provide a new and improved process whereby woody material is reduced for use in the manufacture of pulp with a minimum amount of crushing and bruising of the fibers and in a form which permits rapid and economical reaction with the cooking liquors to produce a pulp of high yield and of high strength for use in the manufacture of improved fibrous structures.

Other objects and advantages of this invention will hereinafter appear and for purposes of illustration, but not of limitation, embodiments of the invention are shown in the accompanying drawing in which:

Figure 1 is a diagrammatic perspective elevational view illustrating the concepts in the reduction of woody materials into wafers for use in the manufacture of pulp in accordance with the practice of this invention;

Figure 2 is a photomicrograph of the surface of a wafer produced in accordance with the illustrated process of Figure 1;

Figures 3, 4 and 5 represent flow sheets for the preparation of pulp with fibrous elements of the type described.

It has been found, in accordance with the practice of this invention, that when the woody material, such as a wooden block 10, is cut into wafers 11 with a cutting edge 12 held parallel to the grain of the wood but adapted to cut across the grain, as distinguished from along the grain, the wafer, as it is being severed, will curl as previously described but curling will occur lengthwise along the axis substantially parallel to the grain of the wood so that little, if any, stresses are imposed on the cellulosic fibers which might result in the damage or crushing thereof. As a result, the fibers remain in condition to resist excessive attack by the cooking liquors and they retain their original characteristics for use in the manufacture of an improved pulp and the manufacture of fibrous structures of greater strength and uniformity at lower cost.

As will be apparent from the photomicrograph of the wafers 11 severed in the manner described from the wooden block 10, very little damage has been found to occur to the fibers on the cut surface of the wafer. The vast differences in pulp formed as between the use of crushed chips and uncrushed chips of wood and as between chips and wafers prepared in accordance with the practice of this invention can be illustrated by the results listed in the following table which compares the pulps formed of crushed and uncrushed chips of Idaho spruce and the pulps of uncrushed chips and wafers of Eastern spruce, all of which have been uniformly processed in accordance with the flow sheet outlined in Figure 3. The results

recorded in the following table were determined in accordance with the standard methods of testing of the Technical Association of the Pulp and Paper Industry.

*Evaluation of beaten pulp from wafers  
and from chips*

| Sample                         | Percent Yield |         | Bulk,<br>cc./g. | Burst,<br>metric | Tear,<br>metric | Tensile,<br>m. | Folds,<br>No. | Screen classification |                 |                    |
|--------------------------------|---------------|---------|-----------------|------------------|-----------------|----------------|---------------|-----------------------|-----------------|--------------------|
|                                | Total         | Rejects |                 |                  |                 |                |               | Retained<br>28 mesh   | 28/200'<br>mesh | Passed<br>200 mesh |
| Uncrushed Chips, I. S. ....    | 35.0          | 4.0     | 1.27            | 121              | 103             | 15,100         | -----         | 88.9                  | 7.9             | 3.2                |
| 0.04" thick wafers, I. S. .... | 39.0          | 0       | 1.25            | 125              | 126             | 15,600         | -----         | 87.4                  | 9.3             | 3.1                |
| 0.01" thick wafers, I. S. .... | 39.5          | -----   | 1.21            | 115              | 99              | 14,200         | -----         | 77.7                  | 16.4            | 5.9                |
| Uncrushed Chips, E. S. ....    | (48)          | -----   | 1.18            | 116              | 83              | 13,600         | 4,801         | 71.8                  | 17.8            | 10.4               |
| Crushed Chips, E. S. ....      | (48)          | -----   | 1.17            | 42               | 50              | 7,960          | 245           | 17.5                  | 71.1            | 11.4               |

E. S. = Eastern spruce.  
I. S. = Idaho spruce.

It will be apparent from the results that a three-fold increase in burst strength and better than a 60 percent increase in tear and tensile strength is achieved with the use of uncrushed chips as compared to crushed chips of the types which have heretofore been prepared for use in the pulp and paper industry. Also a 20-fold increase in the number of folds is secured with pulp formed of uncrushed chips of Eastern spruce. These results fully confirm the work previously noted, of the Canadian Forest Products Laboratory.

With the establishment of the fact that deterioration of the pulp results primarily from the presence of crushed fibers rather than being dependent entirely on the particle size of the wooden material fed into the cooking liquor, it became desirable to achieve means whereby such uncrushed wooden elements could be produced in an efficient and practical manner and preferably in a form adapted for use in the preparation of pulp by the usual cooking processes substantially completely to reduce the wooden elements to pulp without excessive attack and without uncooked portions which otherwise would have to be discarded as waste.

As previously described, wooden wafers substantially free of bruises and damage by crushing can be produced by cutting the wood with a cutting edge held parallel to and advanced across the grain to sever the wafers from the wooden block. In the manufacture of such wafers, it is preferred to score the wood transversely to the grain to define the length of the wafers in situ and then to sever the wafer as an entity from the scored surface of the wood with cutting edges held substantially parallel to the grain and to cut across the grain. Alternatively, the wafers may be economically produced in an efficient manner by means of alternate scalloped and straight edged knives having their main cutting edges held parallel to the grain and adapted to pass across the grain of the wood. Suitable waferizers for use in the reduction of wooden blocks into elements for pulping are described in my copending applications Ser. No. 375,152, Ser. No. 344,089, and Ser. No. 383,893. The apparatus described in the latter application is capable of the very large capacity desired for pulp manufacture, such for example as better than 200 tons of wood per day.

It will also be apparent from the previous table that the pulp secured from wafers prepared in the manner described is superior to pulp prepared of chips which have been carefully formed to prevent crushing. Advantages have been found not only to result in the improved properties of the pulp and the fibrous structures formed thereof but the controlled and uniform dimension of the wafers enables more rapid and more uniform digestion with the cooking liquors to the end that the yield is greatly improved and rejects in the form of chips which have not been cooked are substantially completely avoided.

Various processes well-known to the trade may be used to convert the wafers into pulp for use in the manufacture of fibrous structures. Figure 3 shows a schematic

process for preparing pulp in accordance with the practice of this invention. Figure 4 shows another schematic process for preparing pulp whereby the cooking chemical

20 is added to the wafers and the wafers and chemical are thereafter introduced together into a cooking chamber through a pressure seal. The material progresses along and through the cooking chamber and immerses through another seal to be washed for removal of the cooking 25 chemicals, as in conventional practice.

Figure 5 illustrates a modification of the process outlined in Figure 4. In this process, the wafers are first impregnated with the cooking liquor whereby absorption 30 occurs very uniformly and rapidly, especially if the liquor is hot. The excess liquor is drained from the wafers and they are thereafter subjected to heat and pressure in a closed chamber for a period of time sufficient to permit the residual liquor to cook the woody material to the desired degree. The wafers are thereafter removed from 35 the cooking vessel and washed.

Various modifications may be made in addition to those 40 described without departing from the spirit of the invention. For instance, in the systems illustrated in Figures 4, 5 or 6, the cooking may be accomplished within a steam chamber equipped with a rubbing or disintegrating means, such as a pair of discs, paddles or screws, well known in the art.

Because of the gradual depletion of our forests, it has 45 become desirable to make use of pulping processes which provide for higher yield. One such process which is readily available for use with wafers prepared in accordance with this invention comprises a "semi-chemical" process wherein the woody chips are given a relatively 50 mild cook in which the percentage of active chemical, the time or temperature is restricted so that their yield of pulp will be in excess of 60 percent. The partially 55 softened chips are then disintegrated by various suitable refining means well known in the art. It will be evident that a wafer produced in the manner described, when 60 softened by cooking and then rubbed, will have a decided 65 preference for separating along the grain into long slender fiber bundles and ultimate fibers, and it may be so reduced by a very gentle mechanical action, requiring little power and doing very little damage to the fibrous elements. A semi-cooked chip of the type hitherto used has, after cooking, a hard resistant interior which must be mashed and cut in present semi-chemical processes in order to reduce it, with the result that by the time the chip has been disintegrated, the product consists of excessively short fibers and debris capable of use only in forming a relatively weak and inferior product.

As a result, the use of wafers instead of chips of the type heretofore produced for the manufacture of pulp by a semi-chemical process provides marked advantages, even in those processes which rely upon the wood particles being defibered as they are softened under steam pressure in such equipment as the Asplund defibrator, especially if used in conjunction with a continuous pre-cooker, as is now common practice.

It will be apparent further from the table previously 75 set forth that the pulping process depends in part upon

the thickness of the wafers cut. The preferred thickness of wafers is in the order of about 0.03 to 0.07 inch but the thickness may be varied without interfering with the process other than to lengthen the time necessary for suitable penetration of the cooking liquor sidewise into the fibers as the thickness of the wafer is increased. However, it is undesirable to make use of wafers having a thickness less than 0.01 inch or greater than 0.1 inch. A convenient length of the wafer for purposes of digestion is about 2.5 inches. Since the liquor penetrates along the grain about fifty to one hundred times faster than it does across the grain, a ratio of length to thickness of about 50 or more is desirable. When very sharp knives are used, the wafers can be cut thinner if desired to speed up the absorption of the cooking liquor and the lengths of the wafers may vary in amounts convenient for handling but it is undesirable to make use of wafers having lengths greater than 5 inches.

It will be evident from the foregoing that there is provided a process for the reduction of woody material into elements capable of use in the production of high quality pulp wherein the strengths of the fibers remain substantially intact as a result of the reduction of the woody material without deterioration of the fibers in the reduction process as by crushing or bruising. It will be evident further that the process of the type described for the reduction of woody material produces wafers of a controlled dimension for most efficient penetration of the cooking liquors to enable uniform and complete reduction to pulp thereby to eliminate waste and to minimize attack on the pulp fibers during the cooking process.

It will be understood that changes may be made in the details of production of the wooden wafers within the limitations described and the processing thereof into pulp without departing from the spirit of the invention, especially as defined in the following claims.

I claim:

1. In the method of pulping wood, the steps of reducing blocks of wood into wafers of substantially uniform dimension by cutting the face of the wooden block with cutting edges parallel to and moved across the grain into wafers having a width corresponding to the width of the individual cutting edges, a thickness ranging from 0.01 to 0.1 inch and a length up to 5 inches, said wafers being produced without crushing or bruising, treating the wafers with cooking liquor, and then reducing the cooked wafers into pulp.

2. In the method of pulping wood, the steps of cutting the wood in one face of a block with cutting edges parallel to and moved across the grain into wafers having a thickness of 0.01 to 0.1 inch and of relatively uniform length and width whereby the fibers in the wafers remain relatively free of deterioration by crushing and bruising, then cooking the wafers, and reducing the cooked wafers to a pulp.

3. In the method of pulping wood, the steps of reducing the wood for chemical cooking to form pulp by cutting the wood across one face with cutting edges parallel to and moved across the grain into wafers having a thickness ranging from 0.01 to 0.07 inch whereby the fibers in the wafers remain relatively free of deterioration by crushing and bruising, treating the wafers with an acid cooking liquor and then reducing the cooked wafers into pulp.

4. In the method of pulping wood, the steps of reducing blocks of wood for chemical cooking to form pulp by cutting the blocks in one face with cutting edges parallel to and moved across the grain into wafers having a thickness within the range of 0.01 to 0.1 inches and a length greater than about fifty times the thickness but less than five inches whereby the fibers in the wafers remain relatively free of deterioration by crushing and bruising, treating the wafers with a cooking liquor, and then reducing the cooked wafers into pulp.

5. The method of pulping wood comprising reducing

the wood into wafers of substantially uniform dimension by cutting a block of wood with cutting edges parallel to and moved across the grain into wafers of uniform dimension whereby the fibers in the wafers remain relatively free of deterioration by crushing and bruising, treating the wafers with a cooking liquor, and then reducing the cooked wafers into pulp.

6. In the method of pulping wood, the steps of reducing blocks of wood into wafers of substantially uniform dimension by cutting the face of the wooden block with cutting edges parallel to and moved across the grain into wafers having a width corresponding to the width of the individual cutting edges, a thickness ranging from 0.01 to 0.1 inch and a length about fifty times the thickness but less than 5 inches, mildly cooking the wafers in a semi-chemical process in which the active chemicals and the time and temperatures are controlled partially to soften the bonding agent holding the fibers together in the wafer, and subjecting the partially cooked wafers to gentle mechanical action for separation of the fibers along their grain without damage to the fibrous elements to form pulp fibers.

7. In the method of pulping wood, the steps of reducing blocks of wood into wafers of substantially uniform dimension by cutting the face of the wooden block with cutting edges parallel to and moved across the grain into wafers having a width corresponding to the width of the individual cutting edges, a thickness ranging from 0.01 to 0.1 inch and a length up to 5 inches, treating the wafers under controlled conditions of time, temperature and with chemicals partially to cook the wafers, and rubbing the partially cooked wafers to separate the fibers along the grain without damage to the fibrous elements to form the pulp fibers.

8. In the method of pulping wood, the steps of reducing the wood by chemical and mechanical treatment to form pulp by cutting the wood with a cutting edge parallel to and moved across the grain into wafers of substantially uniform thickness whereby the fibers extend longitudinally in the wafer and remain relatively free of deterioration by crushing and bruising, mildly cooking the wafers in a semi-chemical process in which the active chemicals and the time and temperature are controlled partially to soften the bonding agent securing the fibers one to another in the wafer, and subjecting the partially cooked wafers to a gentle mechanical action to effect separation of fibers along their grain without damage to the fibrous elements to form pulp fibers.

9. In the method of pulping wood, the steps of cutting the wood in one face of a block with cutting edges parallel to and moved across the grain to form wafers having a relatively uniform length ranging from 0.5 to 5.0 inches and a relatively uniform thickness ranging from 0.01 to 0.1 inch whereby the fibers in the cut wafers remain relatively free of deterioration by cutting and bruising, treating woody material comprising such wafers with a chemical solution under controlled conditions of concentration, time and temperature to soften the woody wafers, and then reducing the treated wafers to pulp.

10. The method as claimed in claim 9 wherein the chemical treatment of the wafers and their reduction to pulp is performed as a continuous operation.

#### References Cited in the file of this patent

#### UNITED STATES PATENTS

|           |              |                |
|-----------|--------------|----------------|
| 1,982,130 | Wollenberg   | Nov. 27, 1934  |
| 2,323,194 | Beveridge    | June 29, 1943  |
| 2,509,642 | Horsak       | May 30, 1950   |
| 2,655,189 | Clark        | Oct. 13, 1953  |
| 2,689,092 | Clark et al. | Sept. 14, 1954 |

#### OTHER REFERENCES

The Effect of Chipping on the Suitability of Wood for Sulphite Pulping by Green from Pulp & Paper Magazine of Canada, pages 123-126, Feb. 1940.